

June 6, 1950

H. E. OLES

2,510,598

METHOD OF MAKING IRON CORES

Filed Dec. 12, 1944



Fig. 3



Fig. 4



Fig. 6



Fig. 5



INVENTOR.

Herbert E. Oles  
BY  
Chester F. Carlson

ATTORNEY

## UNITED STATES PATENT OFFICE

2,510,598

## METHOD OF MAKING IRON CORES

Herbert E. Oles, Indianapolis, Ind., assignor to  
 P. R. Mallory & Co., Inc., Indianapolis, Ind., a  
 corporation of Delaware

Application December 12, 1944, Serial No. 567,850

4 Claims. (Cl. 154—80)

1

The present invention relates to the art of forming ferromagnetic core members, and, more particularly, to a novel method of making iron cores from fine-gauge ferromagnetic wire, and to the products of such method.

It is already known to produce a flexible fabric or web including warp strands of textile material and weft strands of a suitable paramagnetic material, such as for example iron wire of appropriate thickness. This fabric or web was wound up into a core body of appropriate shape, characterized by the presence of a large number of parallel-spaced fine ferromagnetic strands. Cores provided in accordance with this method had the advantage of low eddy current losses but were otherwise not particularly efficient in view of their relatively low "space factor."

It is one of the principal objects of the present invention to improve the iron cores of the described generic type and particularly to increase the "space factor" thereof, that is, to increase the proportion of the core volume occupied by the ferromagnetic wire to the total volume of the core.

It is another object of the present invention to provide a novel type of flexible fabric constituted of warp strands of electrically insulating diamagnetic material and of weft strands of ferromagnetic material, the said warp strands being soluble in a suitable solvent so that upon winding up the fabric into a core structure, the warp strands may be dissolved and the remaining body compressed and consolidated thereby to increase the space factor of the finished product.

It is a further object of the invention to provide a novel and improved method of forming iron cores in which warp strands of an electrically insulating thermoplastic diamagnetic material are combined by weaving with weft strands of a paramagnetic material to constitute a fabric subsequently wound up on a core, the wound core structure being subjected to heat and pressure to cause the thermoplastic diamagnetic material to flow, whereby the core structure is consolidated and the space factor thereof is increased.

The invention also contemplates a novel type of core structure comprising a bundle of substantially parallel-spaced iron wires of greatly reduced diameter bonded together by means of thermoplastic diamagnetic materials which is simple in construction, has excellent physical properties, such as high space factor and low eddy current losses, and which may be readily manufactured on a quantity production scale at a low cost.

Other and further objects and advantages of

2

the present invention will become apparent from the following description, taken in conjunction with the accompanying drawing, in which:

Fig. 1 illustrates the weaving pattern of a ferromagnetic fabric embodying the present invention; the thickness of the several strands and the spacing thereof being greatly exaggerated for reasons of clarity;

Fig. 2 depicts a section taken on line 2—2 of Fig. 1;

Fig. 3 shows a ferromagnetic core of cylindrical shape wound up from the fabric of the invention;

Fig. 4 is a diagrammatic view showing the treatment of the wound core body by means of a suitable solvent bath;

Fig. 5 is a similar view illustrating the consolidating step in the method of the invention including the application of pressure with or without the simultaneous application of heat to the preformed core body; and

Fig. 6 is a perspective view of the finished core.

While a preferred embodiment of the invention is described herein, it is contemplated that considerable variation may be made in the method of procedure and the construction of parts without departing from the spirit of the invention. In the following description and in the claims, parts will be identified by specific names for convenience, but they are intended to be as generic in 30 their application to similar parts as the art will permit.

Referring now more particularly to Figs. 1 and 2 of the drawing, reference character 10 denotes the warp threads or strands, while reference character 11 denotes the weft thread or strand. The warp strands may be of any suitable electrically non-conductive diamagnetic material, such as for example conjugated polymers, cellulosic materials as natural and regenerated cellulose and ester and ethers thereof, synthetic resins, elastomers, and the like, which are either soluble in a suitable solvent or which are thermoplastic or fusible in character. The weft strand or strands may be of any suitable paramagnetic material such as, for example, iron wire of appropriate thickness, generally less than 0.01 inch in diameter, and is preferably covered or coated with one or more suitable electrically insulating compounds or materials including insulating varnishes, lacquers, natural and synthetic resins, elastomers, cellulosic materials, and the like. Of course, it is desirable to so select the said covering or coating materials for the paramagnetic strands that they are not attacked by the solvent of the warp strands or, if thermoplas-

tic and fusible warp strands are employed, that the said coating materials have a higher temperature of softening or fusion than the warp strands. As it will be seen in Fig. 1, the finished fabric will appear in the form of a band or web which may be produced in any desired width and length in accordance with the specific application which is contemplated. The diamagnetic strands extend longitudinally of the web, while the paramagnetic strand will extend transversely of the web, reversing its direction at alternate edges of the web to constitute selvedge 12, so formed as to prevent raveling.

The ferromagnetic web embodying the invention may be produced by means of conventional weaving procedures and may be stored and shipped in such condition, if desired. The iron cores may be formed from the said web in various ways. For example, the ferromagnetic web may be wound up to constitute a cylindrical or rod-like core body 13, having a slightly larger diameter than the desired core, as this is shown in Fig. 3.

This wound body is now further treated in order to substantially eliminate the warp strands and thereby to increase the space factor. In case the warp strands are soluble in a suitable solvent, the wound core body is introduced into a treating tank 14 having a quantity of the solvent 15 therein so that the core body is fully submerged in the solvent (Fig. 4). After allowing the solvent to act upon the core body for a sufficient length of time, most of the warp strands will be dissolved or at least considerably softened. The core body is now removed from the solution and is inserted between suitably formed pressure jaws 16 and 17 (Fig. 5). By pressing the said jaws or pressure dies together, the remaining portion of the dissolved or softened warp strands will be squeezed out and only the ferromagnetic weft strands will remain in a strongly consolidated and condensed position. At the same time, the dimensions of the core body will be reduced to those of the desired core. While most of the material of the warp strands will be removed, a small residual amount thereof will be instrumental in permanently bonding the wound structure and will prevent unwinding thereof. It has been found that the finished core structure has excellent magnetic properties, low eddy current losses, and a very high space factor.

As an alternative of the method of the invention, when the warp strands are constituted of a thermoplastic or fusible material, the solvent applying step may be omitted and heat and pressure may be simultaneously applied to the wound core structure by means of the apparatus shown in Fig. 5. In this case, jaws 16 and 17 are heated, for example by means of an electric heating element (not shown), to a temperature sufficient to cause fusion or at least softening of the thermoplastic material of the warp strands. The simultaneous application of heat and pressure will cause the warp strands to soften and to flow so that their major portion will be squeezed out of the wound core body, while their remaining portion upon cooling will permanently bond the weft strand or strands into an integral body of reduced dimensions. The core structure obtained in this manner is shown in Fig. 6 and is likewise characterized by low eddy current losses and a high space factor.

It will be noted that the principles of the invention provide various important advantages. Of these the most important is that iron cores

of a great variety of shapes and sizes may be readily built up from ferromagnetic wire of very small diameter, without the difficulties heretofore encountered in building up cores from fine wire by means of bundling, and the like procedures.

It is also to be observed that the cores embodying the invention substantially eliminate the diamagnetic strands from the finished core structure so that the warp strands do not detrimentally affect the space factor of the finished core.

Moreover, the methods of the invention are very simple and may be readily applied to the quantity production of iron cores from fine-gauge iron wire without requiring any expensive or complicated special equipment.

Although the present invention has been disclosed in connection with a few preferred embodiments thereof, variations and modifications may be resorted to by those skilled in the art without departing from the principles of the present invention. Thus, cores having other than a solid cylindrical shape may be made by substantially the same method, such as tubular cores, and C, I or H-shaped cores. In some cases it may be found advantageous to reverse the relative position of the diamagnetic and paramagnetic strands and to make the warp strands of paramagnetic material and the weft strand of diamagnetic material. All these variations and modifications are considered to be within the true spirit and scope of the present invention, as disclosed in the foregoing description and defined by the appended claims.

What is claimed is:

1. The method of forming core structures for electromagnetic devices which comprises providing a web with warp strands of relatively electrically-non-conductive diamagnetic material and weft strands of a wire of ferrous material, winding up a predetermined length of said web to constitute a core, subjecting said core to a solvent treatment to bring the warp strands at least into a semi-fluid state, and subsequently applying pressure to said core to eliminate the major portion of the material of the warp strands and to obtain a compacted structure substantially consisting of closely spaced ferrous weft strands bonded together by the remainder of the material of said warp strands.

2. The method of forming core structures for electromagnetic devices which comprises providing a web with warp strands of a diamagnetic dielectric material and weft strands of a wire of ferrous material covered by a thin electrically insulating layer, rolling up a predetermined length of said web to constitute a body slightly larger in diameter than that of the desired core, subjecting the said body to a solvent treatment adapted to convert the warp strands at least into a semi-fluid state without substantially attacking the insulating layer of the weft strands, and applying pressure to said body to eliminate the major portion of the material of the warp strands and to obtain a compacted core structure of the desired size substantially consisting of closely spaced ferrous weft strands bonded together by the remainder of the material of said warp strands.

3. The method of forming core structures for electromagnetic devices which comprises providing a web with warp strands of a relatively electrically non-conductive diamagnetic material soluble in a suitable solvent and weft strands of a ferrous material, rolling up a predetermined length of said web to constitute a core, treating

said core with a solvent to dissolve and to remove at least the major portion of the material of the warp strands therein, and subsequently applying pressure to said core to substantially eliminate air spaces therefrom and to obtain a dense core structure consisting of closely spaced ferrous weft strands bonded together by the remainder of the material of said warp strands.

4. The method of forming core structures for electromagnetic devices which comprises providing a web with warp strands of a diamagnetic material soluble in a suitable solvent and weft strands of a ferrous material coated with an electrical insulating material, rolling up a predetermined length of said web to constitute a body larger in diameter than that of the desired core, treating said body with a liquid which is a solvent for the said warp strands and substantially a non-solvent for the coating of the said weft strands, and subsequently compressing the said body to squeeze out the major portion of the material of the warp strands to provide a core structure of the desired dimensions character-

ized by a high space factor and low eddy current losses, said core structure consisting of closely spaced ferrous weft strands electrically insulated from each other by coatings of said insulating material and bonded together by the remainder of the material of said warp strands.

HERBERT E. OLES.

#### REFERENCES CITED

10 The following references are of record in the file of this patent:

#### UNITED STATES PATENTS

| Number    | Name      | Date           |
|-----------|-----------|----------------|
| 1,231,588 | Frederick | July 3, 1917   |
| 1,323,039 | Frederick | Nov. 25, 1919  |
| 1,697,142 | Roller    | Jan. 1, 1929   |
| 1,742,018 | Wermine   | Dec. 31, 1929  |
| 1,903,960 | Dreyfus   | Apr. 18, 1933  |
| 2,014,399 | Sprague   | Sept. 17, 1935 |
| 2,202,013 | Loughheed | May 28, 1940   |
| 2,218,669 | Whipple   | Oct. 22, 1940  |